

# United States Patent [19]

Hinata et al.

[11] 3,873,324

[45] Mar. 25, 1975

[54] **SPECTRALLY SENSITIZED SILVER HALIDE PHOTOGRAPHIC EMULSION**

[75] Inventors: **Masanao Hinata; Haruo Takei; Keisuke Shiba**, all of Kanagawa, Japan

[73] Assignee: **Fuji Photo Film Co., Ltd.**, Kanagawa, Japan

[22] Filed: **Feb. 28, 1974**

[21] Appl. No.: **447,114**

[30] **Foreign Application Priority Data**

Feb. 28, 1973 Japan ..... 48-23987

[52] U.S. Cl. .... **96/124, 96/100**

[51] Int. Cl. .... **G03c 1/14**

[58] **Field of Search** ..... 96/124, 137, 100

[56]

## References Cited

### UNITED STATES PATENTS

|           |         |                    |        |
|-----------|---------|--------------------|--------|
| 3,666,480 | 5/1972  | Shiba et al. ....  | 96/124 |
| 3,672,898 | 6/1972  | Schwan et al. .... | 96/124 |
| 3,702,251 | 11/1972 | Sato et al. ....   | 96/124 |
| 3,799,783 | 3/1974  | Hill et al. ....   | 96/124 |

*Primary Examiner*—J. Travis Brown

*Attorney, Agent, or Firm*—Sughrue, Rothwell, Mion, Zinn & Macpeak

[57] **ABSTRACT**

A silver halide emulsion spectrally sensitized with a combination of a cyanine dye of the general formula (I) as hereinafter defined and a cyanine dye of the general formula (II) as hereinafter defined and having spectral sensitivity in the wave length region ranging from 580 nm to 640 nm.

**13 Claims, 18 Drawing Figures**

PATENTED MAR 25 1975

3,873,324

SHEET 1 OF 4



FIG. 1



FIG. 2



FIG. 3



FIG. 4



FIG. 5



FIG. 6

SHEET 2 OF 4



FIG. 7



FIG. 8



FIG. 9



FIG. 10



FIG. 11



FIG. 12

PATENTED MAR 25 1975

3,873,324

SHEET 3 OF 4



**FIG. 13**



**FIG. 14**



**FIG. 15**



**FIG. 16**



**FIG. 17**

PATENTED MAR 25 1975

3,873,324

SHEET 4 OF 4



FIG. 18

# SPECTRALLY SENSITIZED SILVER HALIDE PHOTOGRAPHIC EMULSION

## BACKGROUND OF THE INVENTION

## 1. Field of the Invention

The present invention relates to a silver halide photographic emulsion which is spectrally sensitized in a specific wave-length region by supersensitization and, more particularly, it is concerned with a silver halide photographic emulsion spectrally sensitized in a wavelength region of from 580 nm to 640 nm.

## 2. Description of the Prior Art

Commonly used photographic light-sensitive materials are provided with a suitable spectral sensitization distribution ranging over the visible wave-length region to which the human eye is sensitive. In order to impart more suitable color reproducibility, more appropriate sensitization distribution is required. Therefore, "combinations showing supersensitization" comprising two

A further object of the present invention is to selectively find supersensitizing dyes which, when incorporated in one layer of a multi-layered light sensitive material to spectrally sensitize the layer selectively so as 5 to attain the abovedescribed objects of the present invention, do not diffuse into adjacent layers to cause sensitization therein.

A still further object of the present invention is to find sensitizing dyes which are more selective, which cause less color stain after development-processing and which cause less reduction in sensitivity even upon storage after production of the light sensitive material (spectrally sensitized by the dyes).

## SUMMARY OF THE INVENTION

The above-described objects can be attained as follows, i.e., by incorporating a supersensitizing combination of at least one carbocyanine dye represented by the following general formula (I):



or more sensitizing dyes are being studied and selected for use.

From the standpoint of obtaining excellent color reproducibility, it is not preferable to impart high sensitivity too far in the longer wave length region, e.g., longer than 660 nm (wave length of the sensitization maximum) or, conversely, to impart sensitivity only in a too short wave length region, e.g., less than 580 nm (wave length of the sensitization maximum).

However, in the conventional spectrally sensitizing art, it has been difficult to selectively increase the sensitivity in the wave length region ranging from 580 nm to 640 nm and the solution of this problem has been an important subject in this art.

35 wherein  $Z_1$  represents the atoms necessary to form a benzothiazole ring, a benzoselenazole ring, a  $\beta$ -naphthothiazole ring or a  $\beta$ -naphthoselenazole ring;  $Z_2$  represents the atoms necessary to form a benzoselenazole ring; A represents a hydrogen atom or an alkyl group;  
 40  $R_1$  and  $R_2$  each represent an alkyl group or a substituted alkyl group, at least one of  $R_1$  and  $R_2$  being a hydroxyalkyl group, a carboxy-substituted alkyl group or a sulfo-substituted alkyl group;  $X_1$  represents an acid anion group; and  $m$  represents 1 or 2 and, when the dye  
 45 forms an internal salt (betaine-like structure),  $m$  represents 1; and at least one carbocyanine dye represented by the general formula (II):



It is, therefore, an object of the present invention to provide a novel supersensitizing combination to selectively increase the sensitivity in the wave length region ranging from 580 nm to 640 nm.

Another object of the present invention is to provide a supersensitizing combination which mitigates the reduction in sensitivity experienced in conventional combinations of supersensitizing dyes.

65 wherein  $Z_3$  and  $Z_4$  each represent the atoms necessary to form a halogen-substituted benzimidazole nucleus;  $R_3$  and  $R_4$  each represents an alkyl group or a substituted alkyl group, at least one of  $R_3$  and  $R_4$  being a hydroxyalkyl group, a carboxy-substituted alkyl group or a sulfo-substituted alkyl group;  $X_2$  represents an acid anion; and  $n$  represents 1 or 2 and, when the dye forms an internal salt,  $n$  represents 1.

## BRIEF DESCRIPTION OF THE DRAWINGS

FIGS. 1 - 17 are spectrograms of photographic materials as described in the Examples and FIG. 18 shows the per cent transmission curve of the filters used in the Examples.

## DETAILED DESCRIPTION OF THE INVENTION

Suitable examples of substituents which can be present on the  $Z_1$  or  $Z_2$  containing heterocyclic nucleus are a halogen atom (e.g., chlorine, fluorine, bromine), a lower alkyl group preferably having no more than 4 carbon atoms in the carbon chain (e.g., methyl, ethyl, etc.), an alkoxy group (e.g., methoxy, ethoxy, etc.), an alkoxy carbonyl group (e.g., methoxycarbonyl, etc.), a trifluoromethyl group, a hydroxy group and a carboxy group.

In the general formulae (I) and (II) which represent the sensitizing dyes to be used in the present invention, the heterocyclic ring formed by  $Z_1$  includes, e.g., benzothiazole, 5-chlorobenzothiazole, 5-bromobenzothiazole, 5-fluorobenzothiazole, 5-methylbenzothiazole, 5-methoxybenzothiazole, 5-methylcarbonylbenzothiazole, 5-methoxycarbonylbenzothiazole, 5-carboxybenzothiazole, 5-hydroxybenzothiazole, 5-trifluoromethylbenzothiazole, 5-cyanobenzothiazole, 5,6-dimethylbenzothiazole, 5,6-dimethoxybenzothiazole, 5,6-dichlorobenzothiazole,  $\beta$ -naphthothiazole, benzoselenazole, 5-chlorobenzoselenazole, 5-bromoselenazole, 5-methylbenzoselenazole, 5-methoxybenzoselenazole,  $\beta$ -naphthoselenazole ring and the like.

The heterocyclic ring formed by  $Z_2$  includes, e.g., a benzoselenazole, 5-chlorobenzoselenazole, 5-bromobenzoselenazole, 5-methylbenzoselenazole, 5-methoxybenzoselenazole ring, and the like.

The heterocyclic ring formed by  $Z_3$  or  $Z_4$  includes chlorine, bromine, fluorine and iodine substituted, preferably chlorine substituted, benzimidazole rings, e.g., 1-methyl-5-chlorobenzimidazole, 1-methyl-5-fluorobenzimidazole, 1-methyl-5,6-dichlorobenzimidazole, 1-ethyl-5-chlorobenzimidazole, 1-ethyl-5-fluorobenzimidazole, 1-methyl-5,6-dichlorobenzimidazole, 1-ethyl-5,6-difluorobenzimidazole, 1-propyl-5-chlorobenzimidazole, 1-propyl-5-fluorobenzimidazole, 1-propyl-5,6-dichlorobenzimidazole, 1-propyl-5,6-difluorobenzimidazole, 1-allyl-5-chlorobenzimidazole, 1-allyl-5,6-dichlorobenzimidazole, 1-allyl-5,6-difluorobenzimidazole, 1-phenyl-5-chlorobenzimidazole, 1-phenyl-5-fluorobenzimidazole, 1-phenyl-5,6-dichlorobenzimidazole, 1-phenyl-5,6-difluorobenzimidazole ring, 1-acetoxyalkyl (e.g., propyl, etc.)-5,6-dichlorobenzimidazole, 1-hydroxyalkyl (e.g., ethyl, etc.)-5,6-dichlorobenzimidazole, and the like.

$R_1$ ,  $R_2$ ,  $R_3$  and  $R_4$  each represents an alkyl group such as an unsubstituted alkyl group (e.g., a methyl group, an ethyl group, a propyl group), a hydroxyalkyl group (e.g., a 2-hydroxyethyl group, a 3-hydroxypropyl group, etc.), a carboxy-substituted alkyl group (e.g., a 2-carboxyethyl group, a 3-carboxypropyl group, a 4-carboxybutyl group, etc.), a sulfo-substituted alkyl group (e.g., a 2-sulfoethyl group, a 3-sulfopropyl group, a 3-sulfobutyl group, a 2[3-sulfopropoxy]ethyl

group, a 2-hydroxy-3-sulfopropyl group, a 3-sulfopropoxyethoxyethyl group, etc.), an acetoxyalkyl group (e.g., acetoxyethyl, etc.), a cyanoalkyl group (e.g., cyanopropyl, etc.), a carbamoylalkyl group (e.g.,  $\beta$ -carbamoylethyl, etc.), a morpholinocarbonylalkyl group [e.g.,  $\beta$ -(4-morpholinocarbonyl)ethyl, etc.], an allyl group, a morpholino sulfonylalkyl group [e.g.,  $\delta$ -(4-morpholinosulfonyl)butyl, etc.], or the like in which the alkyl moiety has, preferably up to 8 carbon atoms.

$X_1^-$  and  $X_2^-$  each represents an acid anion commonly employed in cyanine dye salts, such as an iodide ion, a bromide ion, a chloride ion, a p-toluenesulfonate ion, a benzenesulfonate ion, an ethylsulfate ion, a perchlorate ion, a rhodanide ion, or the like. It is preferred that when two benzimidazole nuclei in the dye of general formula (II) are each substituted with chlorine atom(s), one of  $R_3$  and  $R_4$  is a hydroxyalkyl group, a carboxy-substituted alkyl group or a sulfo-substituted alkyl group and the other is a carbamoylalkyl group, an acetoxyalkyl group, a morpholinocarbonyl group, a cyanoalkyl group, a morpholinosulfonyl group, or an allyl group; or at least one of the nitrogen atoms at the 1-position of the dye of general formula (II) is substituted with an aryl group, an acetoxyalkyl group or an allyl group. Incidentally,



illustrates the above.

A chemical structural feature of the sensitizing dyes represented by the general formula (I) is that they are carbocyanine dyes wherein one or, preferably, two of the substituents connected to the nitrogen atom or atoms in the nitrogen-containing heterocyclic nucleus or nuclei are hydroxyalkyl groups, carboxy-substituted alkyl groups or sulfo-substituted alkyl groups. These dyes show maximum sensitivity in the wave length region ranging from about 600 nm to about 670 nm. Furthermore, they have the feature that, when used in combination with the dye represented by the general formula (II), they increase the spectral sensitivity while maintaining the light sensitivity maximum at a wave length of from about 600 nm to about 630 nm.

A chemical structural feature of the sensitizing dyes represented by the general formula (II) is that they are imidazolocarbocyanines having a hydroxyalkyl group, a carboxy-substituted alkyl group or a sulfo-substituted alkyl group as the substituent connected to the nitrogen atom in the nitrogen-containing heterocyclic nucleus. These dyes show maximum sensitivity in the wave length region ranging from about 570 to about 585 nm and scarcely cause color stain after development processing.

The supersensitizing action by the combined use of the dyes of the present invention strongly counteracts prevention of spectral sensitization due to presence of a color coupler. For example, the desensitization, conventionally experienced in the combined use of a sensitizing dye and a coupler, is extremely small. In addition, since these dyes rarely diffuse into adjacent emulsion layers when applied to one light sensitive layer of a multi-layer light sensitive material, they never sensitize the adjacent layers (silver halide emulsion layers). The above-described effects are never adversely affected

even when a color sensitizer (e.g., 2,2'-cyanine, thia-2'-cyanine, etc.) to increase the green-sensitivity or other color sensitizers (e.g., thiacarbocyanine, etc.) are used in combination.

The supersensitizing technique in accordance with the present invention are useful for the production of ortho-pan type light sensitive emulsions, light sensitive emulsions for mult-layer coupler in the emulsion type color films, particularly, reversal color films and negative color films, for example, as disclosed in U.S. Pat. Nos. 2,698,794; 2,474,293; 2,600,788; 3,311,476; 3,458,315; 3,214,437 and 3,253,924.

Specific examples of the sensitizing dyes which can be used in the present invention are illustrated below. However, the present invention is not limited to the dyes specifically described below.

Specific examples of the dyes represented by the general formula (I):

[I-A]



[I-B]



[I-C]



[I-D]



[I-E]



[I-F]



[I-G]



Specific examples of the dyes represented by the general formula (II):

[II-A]



[II-B]



[III-C][III-D][III-E][III-F][III-G][III-H]

[III-I][III-J][III-K][III-L][III-M][III-N]

[III-O][III-P][III-Q][III-R][III-S][III-T]

Sensitizing dyes used for comparison in demonstrating the effects of the present invention are as follows:

(1)



(2)



(3)



Suitable sensitizing dyes which can be used together with the combination of the dyes of the general formula



(5)



(6)



(7)



lae (I) and (II) of the present invention are described below:

The silver halide photographic emulsions which can be used in the present invention are those produced in a conventional manner and containing silver chloride, silver bromide, silver iodide, silver chlorobromide, silver chloroiodide, silver bromoiodide, silver chlorobromoiodide or mixed silver halide grains thereof, which are precipitated through a single jet method, a double jet method, or a combination of these methods followed by ripening. A preferred silver halide is silver bromoiodide or silver chlorobromoiodide and a preferred mean diameter of the grains (measured by, e.g., a projected area method or a number average method) is from 0.04 micron to 2 microns. Suitable examples of and the preparation thereof are disclosed in U.S. Pat. Nos. 3,217,157; 2,222,264; 3,320,069; 2,592,250; 3,206,313; and 3,367,778 and Belgian Pat. No. 704,255; U.S. Pat. NO. 2,996,382 and Klein and Moisar *Journal of Photographic Science*, volume 12, page 242 et seq., or Markvicki "The Spectral Sensitization of Silver Bromide Emulsion on Different Crystallographic Faces", *Journal of Photographic Science*, volume 13, 1965.

To the silver halide photographic emulsion used in the invention conventionally employed chemical sensitization techniques such as gold sensitization (as described in U.S. Pat. Nos. 2,540,085; 2,597,856; 2,597,915; 2,399,083; etc.), sensitization with a Group VIII metal ion, sulfur sensitization (as described in U.S. Pat. Nos. 1,574,944; 2,278,947; 2,330,206; 2,410,689; 3,189,458; 3,415,649; etc.), reduction sensitization (as described in U.S. Pat. Nos. 2,518,698; 2,419,974; 2,983,610; etc.), or a combination of these sensitization techniques can be employed.

More specifically, the emulsion can contain a sulfur sensitizer such as allylthiocarbamide, thiourea, sodium thiosulfate or cystine; a noble metal sensitizer such as potassium chloroaurate, aurous thiosulfate, or potassium chloropalladate; a reduction sensitizer such as tin chloride, phenylhydrazine or reductone; and the like. Also, the emulsion can contain such a sensitizer as a polyoxyethylene derivative, a polyoxypropylene derivative, a quaternary ammonium group-containing derivative or the like. Furthermore, the emulsion can contain an antifogging agent such as nitrobenzimidazole or ammonium chloroplatinate, and a stabilizing agent such as 4-hydroxy-6-methyl-1,3,3a,7-tetrazaindene.

In addition, the emulsion can contain a hardener, such as formaldehyde, chrome alum, 1-hydroxy-3,5-dichlorotriazine sodium salt, glyoxal, dichloroacrolein, etc., and a coating aid such as saponin, sodium alkylbenzenesulfonate, etc.

Particularly preferred examples of hardeners are aldehyde series compounds such as formaldehyde, glutaraldehyde and halocarboxyaldehydes (e.g., mucochloric acid); ketones such as diacetyl and cyclopentanone; active halogen-containing compounds such as bis(2-chloroethyl)urea, 2-hydroxy-4,6-dichloro-1,3,5-triazine and those compounds as disclosed in U.S. Pat. Nos. 3,288,775 and 2,732,303 and British Pat. Nos.

974,723 and 1,167,207; active olefin-containing compounds such as divinylsulfone, 5-acetyl-1,3-diacryloylhexahydro-1,3,5-triazine and those compounds as disclosed in U.S. Pat. Nos. 3,635,718; 2,232,763; 3,490,911 and 3,642,486 and British Pat. No. 994,869; N-methylol compounds such as N-hydroxymethylphthalimide and those compounds as disclosed in U.S. Pat. Nos. 2,732,316 and 2,586,168; isocyanates as disclosed in U.S. Pat. Nos. 3,103,437; aziridines as disclosed in U.S. Pat. Nos. 3,017,280 and 2,983,611; acid derivatives as disclosed in U.S. Pat. Nos. 2,725,294 and 2,725,295; carbodiimide series compounds as disclosed in U.S. Pat. No. 3,100,704; epoxy compounds as disclosed in U.S. Pat. No. 3,091,537; isooxazoleseries compounds as disclosed in U.S. Pat. Nos. 3,321,313 and 3,543,292; dioxane derivatives such as dihydroxydioxane and dichlorodioxane and inorganic hardeners such as chrom alum and zirconium sulfate, precursors of the above-described materials such as addition compounds of an alkali metal bisulfite and an aldehyde, methylol derivatives of hydrazine, and primary aliphatic nitro alcohols and those compounds as disclosed in U.S. Pat. Nos. 3,288,775; 3,017,280 and 2,983,611 and British Pat. No. 1,167,207. Any of the known surface active agents as a coating aid can be employed and specifically, anionic surface active agents containing acidic groups such as a carboxylic acid group, a sulfonic acid group, a phosphoric acid group, a sulfate group, a phosphate group, etc., amphotolytic surface active agents of carboxylic acid type, sulfonic acid type, sulfate type or phosphate type; nonionic surface active agents of the polyalkyleneoxide series or the polyglycerin series; and natural surface active agents such as saponin, are preferably used. Suitable such materials and the amounts thereof generally suitable for use are disclosed for example, in U.S. Pat. Nos. 2,600,831; 3,068,101; 3,415,649; 3,617,286; 2,271,623; 2,240,472; 2,288,226; 2,739,891; 3,158,484; 3,201,253; 3,210,191; 3,294,540; 3,415,649; 3,441,413; 3,442,654; 3,475,174; 3,545,974; German OLS No. 1,942,665; and British Pat. Nos. 1,077,317 and 1,198,450.

When used in a color photographic light sensitive material, the silver halide emulsion used in the present invention contains a color coupler and a dispersing agent therefor.

Of the color couplers, a cyan coupler is particularly preferred. For example, the phenolic couplers as described in U.S. Pat. No. 2,698,794 and the naphtholic couplers as described in U.S. Pat. No. 2,474,293 are particularly useful. Also, the couplers described in U.S. Pat. No. 2,600,788, British Pat. No. 904,852 and Japanese Patent Publication Number 6031/65, the  $\alpha$ -naphtholic cyan couplers and the phenolic cyan couplers described in, e.g., U.S. Pat. Nos. 3,311,476; 3,458,315; 3,214,437 and 3,253,924 can be used. For example, the couplers represented by the following structural formulae can be used, all of which are known compounds.

(C-1)



(C-2)



(C-3)



(C-4)



(C-5)



(c-6)



(C-7)



(c-8)



(C-9)(C-10)(C-11)(C-12)(C-13)(C-14)(C-15)

(C-16)



(C-17)



(C-18)



Photographic emulsions spectrally sensitized with the dye combinations of the present invention can contain various colloids alone or in combination as vehicles or binding agents. Suitable hydrophilic materials include both naturally-occurring substances such as proteins, for example, gelatin, gelatin derivatives such as phthaloylated gelatin or malonoylated gelatin, cellulose derivatives such as hydroxyethyl cellulose or carboxy methyl cellulose, polysaccharides such as dextran, gum arabic and the like; and synthetic polymeric substances such as water soluble polyvinyl compounds, e.g., polyvinyl alcohol, poly(vinylpyrrolidone), acrylamide polymers, polystyrenesulfonic acid, or other synthetic polymeric compounds such as dispersed vinyl compounds in latex form, and particularly those which increase the dimensional stability of the photographic materials. Suitable synthetic polymers include those described, for example, in U.S. Pat. Nos. 3,142,568; 3,193,386; 3,062,674; 3,220,844; 3,287,289 and 3,411,911. Particularly effective are those water insoluble polymers of alkyl acrylates and methacrylates, acrylic acid, sulfoalkyl acrylates or methacrylates, those which have cross linking sites which facilitate hardening or curing and those having recurring sulfobetaine units as described in Canadian Pat. No. 774,054. As the matting agent which can also be present in the emulsion, there are preferably used silver halide grains of a suitable grain size; inorganic compounds such as silica, strontium barium sulfate, etc.; water-dispersable vinyl polymers such as polymethyl methacrylate, etc. Examples of plasticizers which can be present in the emulsion are waxes such as liquid paraffin, higher fatty acid esters, etc.; polyfluorinated hydrocarbons or derivatives thereof;

silicones such as polyalkylpolysiloxane, polyarylpolysiloxane, polyalkylarylpolysiloxane or the alkylene oxide adduct derivatives thereof; and the like are preferably used.

40 The finished emulsion is applied to a suitable support such as baryta paper, a resin-coated paper, a synthetic paper, a triacetate film, a polyethylene terephthalate film, a glass plate or other plastic bases.

45 These addenda described above are used in an amount to achieve their known function and such can easily be determined by one skilled in the art.

The sensitizing dyes of the general formula (I) and (II) used in the present invention are added as a solution prepared by dissolving the dyes in water or a water-miscible organic solvent such as methanol, ethanol, methyl cellosolve, pyridine or the like.

50 Each of these dyes is used in the amount usually employed in supersensitization, e.g.,  $5 \times 10^{-3}$  mol to  $1 \times 10^{-6}$  mol, preferably  $1 \times 10^{-5}$  mol to  $1 \times 10^{-3}$  mol, per 1 mol of silver. A preferred molar ratio of the amount of the dye represented by the general formula (II) to that of the dye represented by the general formula (I) ranges from 1:10 to 10:1, particularly 1:5 to 5:1 and more particularly 1:3 to 3:1.

55 Also, the dyes to be used in the present invention can be used for spectral sensitization according to German OLS Pat No. 2,104,284 and U.S. Pat. No. 3,649,286.

60 The present invention will now be illustrated in greater detail by reference to the following examples which, however, are not intended to limit the present invention in any way. Unless otherwise indicated, all parts, percents, ratios and the like are by weight.



TABLE 1—Continued

| No. | Dye and Amount<br>Used $\times 10^5$ mol | Dye and Amount<br>Used $\times 10^5$ mol | Dye and Amount<br>Used $\times 10^5$ mol | $S_Y^*$ | $S_R^*$ | $S_B^*$ | Fog  | Spectrogram  |      |
|-----|------------------------------------------|------------------------------------------|------------------------------------------|---------|---------|---------|------|--------------|------|
| 10  | (I - F)                                  | 0.5                                      | —                                        | —       | 68      | 53      | 96   | 0.07         |      |
|     | —                                        | 1                                        | —                                        | —       | 106     | 92      | 92   | 0.07         |      |
|     | —                                        | 2                                        | —                                        | —       | 142     | 130     | 85   | 0.08         |      |
| 10  | —                                        | (II - E)                                 | 1                                        | —       | 140     | 86      | 98   | 0.07         |      |
|     | —                                        | —                                        | 2                                        | —       | 198     | 110     | 90   | 0.08         |      |
|     | (I - F)                                  | 0.5                                      | (II - E)                                 | 4       | —       | 230     | 120  | 88           |      |
| 11  | —                                        | —                                        | 4                                        | —       | 395     | 350     | 92   | 0.08         |      |
|     | (I - A)                                  | 1                                        | (II - E)                                 | 4       | —       | 405     | 358  | 92           | 0.08 |
|     | —                                        | 2                                        | —                                        | —       | 432     | 280     | 96   | 0.08         |      |
| 12  | (2)                                      | 1                                        | (3)                                      | 4       | —       | 438     | 288  | 90           | 0.08 |
|     | —                                        | 2                                        | —                                        | —       | 125     | 75      | 47   | 0.10         |      |
|     | —                                        | —                                        | —                                        | —       | 128     | 80      | 40   | 0.10         |      |
|     | —                                        | —                                        | —                                        | —       | —       | 100     | 0.07 | FIG. 10 - 22 |      |

\* Relative value

## EXAMPLE 2

80 grams of a cyanine coupler, 1-hydroxy-4-maleimido-2-naphthamide, was completely dissolved in a mixed solution of 100 cc of tricresyl phosphate and 50 cc of ethyl acetate. Furthermore, 2 g of sorbitan monolaurate was dissolved therein. The resulting solution was added to a mixture, prepared by adding as an aqueous solution 2.5 g of dodecylbenzenesulfonic acid to 1 kg of a 10 % by weight gelatin, stirred at a high speed and subjected to ultrasonic wave stirring to emulsify. Thus, an emulsion was obtained.

1 kg portions of the silver bromoiodide emulsion prepared according to the method of Example 1 were weighed out in a pot, which was then placed in a 50°C thermostatic bath to melt the emulsions. Methanol solutions of the sensitizing dyes of the present invention and the sensitizing dyes for comparison were added to the emulsion portions in predetermined amounts (as shown in Table 2), mixed and stirred at 40°C, and then left for 15 minutes. To each emulsion portion were added 250 g of the above-described emulsion, 10 cc of a 0.1 % by weight aqueous solution of 4-hydroxy-6-methyl-1,3,3a,7-tetrazaindene, 10 cc of a 1 % by weight aqueous solution of 1-hydroxy-3,5-dichlorotriazine sodium salt and 10 cc of a 1 % by weight aqueous solution of sodium dodecylbenzenesulfonate, and stirred.

Each of the thus finished emulsion portions was applied to a cellulose triacetate film base in a dry thickness of 5  $\mu$  followed by drying. Thus, light sensitive material samples were obtained.

Each of these film samples was cut into strips. One of the strips was wedgewise exposed through a red filter Sc-56 using a sensitometer containing a light source of a color temperature of 5400°K.

This was development-processed at 24°C for 10 minutes in a developer having the following composition followed by washing, hardening, washing and second reversal exposure.

| Composition of the Developer:  |       |
|--------------------------------|-------|
| N-Methyl-p-aminophenol         | 4.5 g |
| Hydroquinone                   | 4.5 g |
| Sodium Sulfite (anhydrous)     | 50 g  |
| Sodium Carbonate (monohydrate) | 30 g  |
| Potassium Bromide              | 1 g   |
| Potassium Thiocyanate          | 2 g   |
| Water to make                  | 1     |

The strip was then color development-processed at 24°C for 15 minutes in a color developer having the following composition followed by washing, bleaching, washing, fixing and washing. Thus, a color positive image was obtained.

| Composition of Color Developer:                                          |       |
|--------------------------------------------------------------------------|-------|
| Benzyl Alcohol                                                           | 6 ml  |
| Sodium Sulfite (anhydrous)                                               | 4 g   |
| Sodium Tertiary Phosphate                                                | 40 g  |
| Sodium Hydroxide                                                         | 1.5 g |
| Potassium Bromide                                                        | 0.5 g |
| Ethylenediamine                                                          | 5 ml  |
| Citrazinic Acid                                                          | 1 g   |
| p-Amino-N-ethyl-N- $\beta$ -methane-sulfonamidoethyl-m-toluidine Sulfate | 11 g  |
| Water to make the total                                                  | 1     |

The density of the thus obtained strips was measured using an S-type densitometer (made by Fuji Photo Film Co. Ltd.) to obtain the relative sensitivity and cyan color fog. The standard point of the optical density to determine the sensitivity was fog + 0.5. The results obtained are shown in Table 2.

Run Nos. 3, 4, 7 and 8 were conducted for comparison.

On the other hand, the one remaining strip was exposed using a grating spectrophotograph having a 2660°K tungsten light source to obtain spectrograms. The thus obtained spectrograms are shown in FIGS. 11 to 17.

From the values given in Table 2 and from the spectrograms obtained, it can be seen that the effects of the combination of dyes of the present invention having supersensitizing action are excellent and are affected by the coupler with difficulty as compared with the comparative dyes.

TABLE 2

| No. | Dye and Amount<br>Used $\times 10^5$ mol |          | Dye and Amount<br>Used $\times 10^5$ mol |          | Dye and Amount<br>Used $\times 10^5$ mol |          | Relative<br>Sensi-<br>tivity | Cyan<br>Fog  | Spectrogram  |
|-----|------------------------------------------|----------|------------------------------------------|----------|------------------------------------------|----------|------------------------------|--------------|--------------|
|     | (I - A)                                  | (II - B) | (I - A)                                  | (II - B) | (I - A)                                  | (II - B) |                              |              |              |
| 1   | —                                        | —        | —                                        | —        | —                                        | —        | 0.07                         | FIG. 11 - 23 | FIG. 11 - 23 |
|     | 1                                        | —        | —                                        | —        | —                                        | —        | 0.07                         |              |              |
|     | 2                                        | —        | —                                        | —        | —                                        | —        | 0.07                         |              |              |
|     | —                                        | (II - B) | 1                                        | —        | —                                        | —        | 0.07                         |              |              |
|     | —                                        | —        | 2                                        | —        | —                                        | —        | 0.07                         |              |              |
|     | —                                        | —        | 4                                        | —        | —                                        | —        | 0.07                         |              |              |
|     | (I - A)                                  | —        | (II - B)                                 | 4        | —                                        | —        | 0.08                         |              |              |
|     | 1                                        | —        | 4                                        | —        | —                                        | —        | 0.08                         |              |              |
|     | 2                                        | —        | 4                                        | —        | —                                        | —        | 0.08                         |              |              |
|     | —                                        | —        | —                                        | (6)      | 1                                        | —        | 0.07                         |              |              |
| 2   | —                                        | —        | —                                        | —        | 2                                        | —        | 0.07                         | FIG. 12 - 26 | FIG. 12 - 26 |
|     | (I - A)                                  | —        | (II - B)                                 | 4        | (6)                                      | 2        | —                            |              |              |
|     | 1                                        | —        | 4                                        | —        | —                                        | —        | 0.08                         |              |              |
|     | 2                                        | —        | —                                        | —        | —                                        | —        | 0.07                         |              |              |
| 3   | —                                        | —        | —                                        | —        | —                                        | —        | 0.07                         | FIG. 12 - 27 | FIG. 12 - 27 |
|     | (I - A)                                  | —        | (II - B)                                 | 4        | (6)                                      | 2        | —                            |              |              |
|     | 1                                        | —        | 4                                        | —        | —                                        | —        | 0.08                         |              |              |
|     | 2                                        | —        | —                                        | —        | —                                        | —        | 0.07                         |              |              |
| 4   | —                                        | —        | —                                        | —        | —                                        | —        | 0.07                         | FIG. 13 - 28 | FIG. 13 - 28 |
|     | (I)                                      | —        | (II - B)                                 | 4        | —                                        | —        | 0.07                         |              |              |
|     | 1                                        | —        | 4                                        | —        | —                                        | —        | 0.08                         |              |              |
|     | 2                                        | —        | —                                        | —        | —                                        | —        | 0.07                         |              |              |
| 5   | —                                        | —        | —                                        | —        | —                                        | —        | 0.07                         | FIG. 13 - 29 | FIG. 13 - 29 |
|     | (I - A)                                  | —        | (II - B)                                 | 4        | —                                        | —        | 0.08                         |              |              |
|     | 1                                        | —        | 4                                        | —        | —                                        | —        | 0.08                         |              |              |
|     | 2                                        | —        | —                                        | —        | —                                        | —        | 0.07                         |              |              |
| 6   | —                                        | —        | (3)                                      | —        | —                                        | —        | 0.07                         | FIG. 14 - 30 | FIG. 14 - 30 |
|     | (I - A)                                  | —        | (3)                                      | —        | —                                        | —        | 0.10                         |              |              |
|     | 1                                        | —        | 4                                        | —        | —                                        | —        | 0.10                         |              |              |
|     | 2                                        | —        | 4                                        | —        | —                                        | —        | 0.10                         |              |              |
| 7   | (I - E)                                  | —        | —                                        | —        | —                                        | —        | 0.07                         | FIG. 14 - 31 | FIG. 15 - 32 |
|     | 1                                        | —        | —                                        | —        | —                                        | —        | 0.07                         |              |              |
|     | 2                                        | —        | —                                        | —        | —                                        | —        | 0.07                         |              |              |
|     | (I - E)                                  | —        | (II - B)                                 | 4        | —                                        | —        | 0.08                         |              |              |
| 8   | (I - E)                                  | —        | (II - B)                                 | 4        | (6)                                      | 2        | —                            | FIG. 15 - 33 | FIG. 15 - 33 |
|     | 1                                        | —        | 4                                        | —        | —                                        | —        | 0.08                         |              |              |
|     | 2                                        | —        | 4                                        | —        | —                                        | —        | 0.08                         |              |              |
|     | (2)                                      | —        | (II - B)                                 | 4        | —                                        | —        | 0.08                         |              |              |
| 7   | (1)                                      | —        | (II - B)                                 | 4        | (6)                                      | 2        | —                            | FIG. 16 - 34 | FIG. 16 - 34 |
|     | 1                                        | —        | 4                                        | —        | —                                        | —        | 0.07                         |              |              |
|     | 2                                        | —        | 4                                        | —        | —                                        | —        | 0.07                         |              |              |
|     | (2)                                      | —        | (II - B)                                 | 4        | —                                        | —        | 0.07                         |              |              |
| 8   | (2)                                      | —        | (3)                                      | 4        | —                                        | —        | 0.09                         | FIG. 16 - 35 | FIG. 16 - 35 |
|     | 1                                        | —        | (3)                                      | 4        | —                                        | —        | 0.09                         |              |              |
|     | 2                                        | —        | 4                                        | —        | —                                        | —        | 0.09                         |              |              |

The combination of sensitizing dyes of the present invention having sensitizing action is useful for spectrally sensitizing a silver halide emulsion using for a red-sensitive layer in color light sensitive materials such as a color negative light sensitive material and a color reversal light sensitive material; a silver halide emulsion for use in a plate-making light sensitive material; and a silver halide emulsion for use in a light sensitive material for microsecond exposure, particularly, a CRT sensitive material, a light sensitive material for holography and a light sensitive material for use in a facsimile system.

In the case of using as a color light sensitive material, it is preferable to provide a magenta or red outer filter above or adjacent to the red-sensitive silver halide emulsion layer obtained by the present invention so as to impart the effect of actually reducing the green-sensitivity in contrast to the red-sensitivity. In order to form such filter layer, the dyes described in Japanese Pat. Nos. 18459/66, 350/68, 13168/68, 22069/64, 98474/71, 42668/71, 42667/71, U.S. Pat. Nos. 3,440,051; 3,468,883; 3,294,539; 3,379,533; 3,352,680; 3,389,994; 3,384,487; 3,423,207; 3,493,375; 3,486,897; 3,481,927; 3,497,502; 55 3,573,289; 3,560,214; 3,615,432; 3,282,699; British Pat. No. 506,385, etc. can be used. In particular, those dyes which selectively absorb light of wave lengths shorter than 570 mm are useful. In addition, the methods described in German OLS No. 2,008,882, U.S. Pat. 60 Nos. 3,425,834; 3,282,699, Belgian Pat. Nos. 682,413; 685,292; 703,939; 627,308, Japanese Pat. Nos. 21766/68, 13498/68, 15896/70, 10254/68, etc. can be employed. These are also employable for preventing irradiation of halation. 65

While the invention has been described in detail and with reference to specific embodiments thereof, it will be apparent to one skilled in the art that various

changes and modifications can be made therein without departing from the spirit and scope thereof.

What is claimed is:

1. A silver halide photographic emulsion containing a supersensitizing combination of at least one sensitizing dye represented by the following general formula (I)



wherein  $Z_1$  represents the atoms necessary to form a benzothiazole ring, a benzoselenazole ring, a  $\beta$ -naphthothiazole ring or a  $\beta$ -naphthoselenazole ring;  $Z_2$  represents the atoms necessary to form a benzoselenazole ring;  $A$  represents a hydrogen atom or an alkyl group;  $R_1$  and  $R_2$  each represents an alkyl group, at least one of  $R_1$  and  $R_2$  being a hydroxylalkyl group, a carboxy-substituted alkyl group or a sulfo-substituted alkyl group;  $X_1$  represents an acid anion group; and  $m$  represents 1 or 2 and, when the dye forms an intramolecular salt,  $m$  represents 1; and at least one sensitizing dye represented by the general formula (II)



wherein  $Z_3$  and  $Z_4$  each represents the atoms necessary to form a halogen-substituted benzimidazole nucleus;  $R_3$  and  $R_4$  each represents an alkyl group, at least one of  $R_3$  and  $R_4$  being a hydroxyalkyl group, a carboxy-substituted alkyl group or a sulfo-substituted alkyl group;  $X_2$  represents an acid anion; and  $n$  represents 1 or 2 and, when the dye forms an intramolecular salt,  $n$  represents 1.

2. The silver halide photographic emulsion as described in claim 1, wherein in the general formula (I)  $Z_1$  forms a  $\beta$ -naphthothiazole ring, a  $\beta$ -naphthoselenazole ring or a benzothiazole or benzoselenazole ring which is unsubstituted or substituted with a methyl group, an ethyl group, a methoxy group, a phenyl group or a chlorine atom at the 5-position;  $Z_2$  forms a benzoselenazole ring which is unsubstituted or substituted with a methyl group, an ethyl group, a methoxy group, a phenyl group or a chloride atom at the 5-position;  $R_1$  and  $R_2$  each is a sulfo-substituted alkyl group, a carboxy-substituted alkyl group or a hydroxyalkyl group; and A is a methyl group.

3. The silver halide photographic emulsion as described in claim 1, wherein at least one of  $R_1$  and  $R_2$  is a sulfo-substituted alkyl group and at least one of  $R_3$  and  $R_4$  is a sulfo-substituted alkyl group.

4. The silver halide photographic emulsion as described in claim 1, wherein in the general formula (II)  $Z_3$  and  $Z_4$  form benzimidazole rings substituted with chlorine atoms or fluorine atoms at the 5, 6, 5' and 6' positions.

5. The silver halide photographic emulsion as described in claim 1, wherein  $R_1$ ,  $R_2$ ,  $R_3$  and  $R_4$  are sulfo-substituted alkyl groups.

6. A color light sensitive material comprising a support having thereon the silver halide photographic emulsion as described in claim 1.

7. The silver halide photographic emulsion as described in claim 1, wherein said alkyl group for  $R_1$  -  $R_4$  is an unsubstituted alkyl group, a hydroxyalkyl group, a carboxy-substituted alkyl group, a sulfo-substituted alkyl group, an acetoxyalkyl group, a cyanoalkyl group, a carbamoylalkyl group, a morpholinocarbonyl group, an allyl group or a morpholinosulfonylalkyl group.

8. The silver halide photographic emulsion as described in claim 1, wherein  $Z_1$  is a benzothiazole, 5-chlorobenzothiazole, 5-bromobenzothiazole, 5-fluorobenzothiazole, 51-methylbenzothiazole, 51-methoxybenzothiazole, 5-methylcarbonylbenzothiazole, 5-methoxycarbonylbenzothiazole, 5-carboxybenzothiazole, 5-hydroxybenzothiazole, 5-trifluoromethylbenzothiazole, 5-cyanobenzothiazole, 5,6-dimethylbenzothiazole, 5,6-dimethoxybenzothiazole, 5,6-dichlorobenzothiazole,  $\beta$ -naphthothiazole, benzoselenazole, 5-chlorobenzoselenazole, 5-bromoselenazole, 5-methylbenzoselenazole, 51-methoxybenzoselenazole or  $\beta$ -naphthoselenazole ring; wherein  $Z_2$  is a benzoselenazole, 5-chlorobenzoselenazole, 5-bromobenzoselenazole, 5-methylbenzoselenazole or 5-methoxybenzoselenazole ring; wherein  $Z_3$  and  $Z_4$  each is a 1-methyl-5-chlorobenzimidazole, 1-methyl-5-fluorobenzimidazole, 1-methyl-5,6-dichlorobenzimidazole, 1-ethyl-5-chlorobenzimidazole, 1-ethyl-5-fluorobenzimidazole, 1-methyl-5,6-dichlorobenzimidazole, 1-ethyl-5,6-difluorobenzimidazole, 1-propyl-5-chlorobenzimidazole, 1-propyl-5-fluorobenzimidazole, 1-propyl-5,6-dichlorobenzimidazole, 1-propyl-5,6-difluorobenzimidazole, 1-allyl-5-chlorobenzimidazole,

1-allyl-5-fluorobenzimidazole, 1-dichlorobenzimidazole, 1-difluorobenzimidazole, 1-phenyl-51-chlorobenzimidazole, 1-phenyl-5-fluorobenzimidazole.

5 1-phenyl-5,6-dichlorobenzimidazole, 1-phenyl-5,6-difluorobenzimidazole ring; wherein said alkyl group for A is a methyl group, an ethyl group, or a propyl group; wherein said  $R_1$  to  $R_4$  each is a methyl group, an ethyl group, a propyl group, a 2-hydroxyethyl group, a 3-hydroxypropyl group, a 2-carboxyethyl group, a 3-carboxypropyl group, a 4-carboxybutyl group, a 2-sulfoethyl group, a 3-sulfopropyl group, a 3-sulfobutyl group, a 2-[3-sulfopropoxy]ethyl group, a 2-hydroxy-3-sulfopropyl group, a 3-sulfopropoxyethoxyethyl group, 15 an acetoxyethyl group, a cyanopropyl group, a  $\beta$ -carbamoylethyl group, a  $\beta$ -(4-morpholinocarbonyl)ethyl group, or a  $\delta$ -(4-morpholinosulfonyl)butyl group.

9. The silver halide photographic emulsion as described in claim 1, including a cyan coupler.

10 20 The silver halide photographic emulsion as described in claim 1, wherein the supersensitizing combination contains anhydro-5,5',9-trimethyl-3,3'-di(3-sulfopropyl)selenacarbocyanine hydroxide and anhydro-5,5',6,6'-tetrachloro-1,1'-diethyl-3,3'-di(3-sulfopropoxyethoxyethyl)benzimidazolocarbocyanine hydroxide mono sodium salt.

11 30 The silver halide photographic emulsion as described in claim 1, wherein the supersensitizing combination contains anhydro-5,5',9-trimethyl-3,3'-di(3-sulfopropyl)selenacarbocyanine hydroxide and anhydro-5,5',6,6'-tetrachloro-1,1',3-triethyl-3'-(3-sulfopropyl)benzimidazolocarbocyanine hydroxide.

12 35 The silver halide photographic emulsion as described in claim 1, wherein the supersensitizing combination contains anhydro-5,5',9-trimethyl-3,3'-di(3-sulfopropyl)selenacarbocyanine hydroxide and anhydro-5-(2-carbamoylethyl)-5,5',6,6'-tetrachloro-1,1'-diethyl-3'-sulfopropyl benzimidazolocarbocyanine hydroxide.

13 40 40 A silver halide photographic emulsion containing a supersensitizing combination of at least one sensitizing dye represented by the following general formula (I)



wherein  $Z_1$  represents the atoms necessary to form a benzothiazole ring, a benzoselenazole ring, a  $\beta$ -naphthothiazole ring or a  $\beta$ -naphthoselenazole ring;  $Z_2$  represents the atoms necessary to form a benzoselenazole ring; A represents a hydrogen atom or an alkyl group;  $R_1$  and  $R_2$  each represents an alkyl group, at least one of  $R_1$  and  $R_2$  being a hydroxyalkyl group; a carboxy-substituted alkyl group or a sulfo-substituted alkyl group; X represents an acid anion group; and m represents 1 or 2 and, when the dye forms an intramolecular salt, m represents 1; and at least one sensitizing dye represented by the general formula (II)



wherein  $Z_3$  and  $Z_4$  each represents the atoms necessary to form a halogen-substituted benzimidazole nucleus;  $R_3$  and  $R_4$  each represents an alkyl group;  $X_2$  represents an acid anion; and  $n$  represents 1 or 2 and, when the

dye forms an intramolecular salt,  $n$  represents 1; with proviso that when two benzimidazole nuclei in the dye of the general formula (II) are each substituted with chlorine atom(s), one of the  $R_3$  or  $R_4$  is a hydroxylalkyl group, a carboxy-substituted alkyl group or a sulfo-substituted alkyl group and the other of  $R_3$  or  $R_4$  is a carbamoylalkyl group, an acetoxyalkyl group, a morpholinocarbonyl group, a cyanoalkyl group, a morpholinosulfonyl group, or an alkyl group, or at least one of nitrogen atoms at the 1-position of the dye of the general formula (II) is substituted with an aryl group, an acetoxyalkyl group or an allyl group.

\* \* \* \* \*

15

20

25

30

35

40

45

50

55

60

65